

## UNITED STATES PATENT OFFICE.

CHARLES D. HALL, OF DETROIT, ILLINOIS.

## POLISHING COMPOUND.

No Drawing.

Application filed June 7, 1926. Serial No. 114,317.

This invention relates to polishing fluids and is particularly intended as a polish for automobile bodies.

This invention has for its primary object 5 the provision, in a manner as hereinafter set forth, of a polishing fluid which will give a clear, hard lustre and will not be greasy or oily, drying rapidly so that dust and grit will not collect upon the finish to which the 10 polish is applied to cut into and ruin the same. No rubbing or polishing is required in connection with the use of this polish and approximately thirty minutes after the application of the same, a dry, hard and glossy 15 finish will result.

The product embodying this invention will be best understood from a consideration of the following detailed description of the same, with the understanding that 20 the invention is not confined strictly to the reading of the specification, but may be changed and modified so long as such changes and modifications mark no material departure from the salient features of the 25 invention as expressed in the appended claim.

The polish embodying this invention comprises a mixture of spar varnish, turpentine, japan drier, black enamel and ether. 30 These ingredients are shaken well together

and thereafter the polish is ready for application.

The preferred proportionate quantities of the ingredients of this formula, are as follows:—Spar varnish, 3 pints; turpentine, 2 35 quarts; japan drier,  $\frac{1}{2}$  pint; black enamel,  $\frac{1}{4}$  ounce; ether, 1 ounce.

The mixture of spar varnish and turpentine makes a fluid easily applicable polish which will readily dry owing to the inclusion in the formula of the japan drier and ether. A hard waterproof and smooth 40 finish will thus result and the black enamel associated with the other ingredients, gives of course, a black lustre to the finish. 45

The application of this polish is very simple, as it may be applied with a piece of soft cloth to the surface, after the surface has been thoroughly washed and dried.

Having thus described my invention what 50 I claim is:—

A polish of the character described, comprising the following ingredients in the approximate set forth proportions:—Spar varnish, 3 pints; turpentine, 2 quarts; japan 55 drier,  $\frac{1}{2}$  pint; black enamel,  $\frac{1}{4}$  ounce; and ether, one ounce.

In testimony whereof, I affix my signature hereto.

CHARLES D. HALL.